

## UNITED STATES PATENT OFFICE.

LUCIEN PAUL BASSET, OF PARIS, FRANCE.

## PROCESS FOR THE DIRECT REDUCTION OF ORES, AND PARTICULARLY OF IRON ORES.

No Drawing.

Application filed February 21, 1923. Serial No. 620,505.

*To all whom it may concern:*

Be it known that I, LUCIEN PAUL BASSET, of 54 Avenue Marceau, Paris, France, chemist engineer, have invented Processes for the 5 Direct Reduction of Ores, and Particularly of Iron Ores, of which the following is a full, clear, and exact description.

In my prior United States Patents Nos. 1,360,711 and 1,372,392, and in my pending 10 United States application filed on the March 10th, 1920, under Serial No. 364,704, there are described various processes for the direct production of iron and its alloys based upon the following principle:

15 The ore to be reduced is mixed with the necessary quantity of coal for effecting the reduction and the whole is heated by means of a flame obtained by the combustion of finely pulverized coal in the quantity of 20 superheated air necessary for causing this combustion to practically give only carbon monoxide.

Under the action of this extremely hot flame, the reaction of the coal on the ore is 25 complete since no reverse reaction can take place, and the metal melts without any possible prejudicial reaction since the flame, and consequently the atmosphere of the furnace does not contain any element capable of yielding oxygen. Owing to this fact, 30 the reduction of the ore is complete and the slag of the furnace is practically free of iron oxide.

The accessory reactions of iron metallurgy in particular also are satisfactory due to these chemical conditions: by the process above set forth, sulphur, for instance, is extracted from the iron as a calcareous slag, since this process prohibits any oxidation 40 of sulphide of calcium and consequently its reincorporation in the metal.

Experience has shown the applicant that in the process which has just been mentioned it might sometimes be advantageous, as far 45 as economy is concerned, to use a heating flame containing a certain proportion of carbonic acid but always less than the proportion of carbon monoxide, in order that the flame can never exert a prejudicial oxidizing action.

The use of such a heating flame is more

economical than that of a flame practically containing only carbon monoxide for the two following reasons:

1. It is no longer necessary to crush the 55 fuel so finely and the quantity of pulverized coal used can be reduced, thereby reducing the expense of the preparation of the fuel.

2. Economy in the consumption of fuel 60 since carbonic acid produces when burning 8080 calories, whilst carbon monoxide produces only 2473 calories.

The process forming the subject-matter of the present invention consists therefore in subjecting the ore, mixed with the quantity of coal necessary for its reduction and to which are added suitable fluxes, to the action of a flame obtained by the combustion of pulverized coal in the necessary quantity of superheated air in order that the combustion 70 produces carbon monoxide and a certain quantity of carbonic acid less than that of carbon monoxide, in such a manner that the oxidizing action exerted by this carbonic acid on iron during the reduction and melting 75 does not reach a prejudicial proportion.

Thus, for instance, if the combustion of the pulverized coal in the superheated air is carried out so as to give, no longer solely carbon monoxide, but 85% of carbon monoxide and 15% of carbonic acid, the reduction of the ore in this case, instead of being total, will amount to 95%, but the loss of metal arising from the oxidizing action of carbonic acid will be largely compensated 80 by the economy resulting from the fact that it is not necessary to so finely pulverize the coal and that the necessary quantity of pulverized coal employed will be less. Moreover, it is to be noted that in this case the 90 temperature of the flame will be a little higher.

It might be therefore to advantage in certain cases to lose a small fraction of reduced metal owing to the economy obtained by the 95 diminution of the quantity of pulverized coal employed and of the greater facility of crushing the latter.

The present process of reduction can be used in the processes described in my prior 100 United States Patents Nos. 1,360,711, 1,372, 392, 1,435,686 and in my pending United

States patent application filed on the March 10th, 1920, under Serial No. 364,704.

Claim:

A process for the reduction of ores and particularly iron ores, which consists in subjecting the ore, mixed with the quantity of coal necessary for its reduction and to which are added suitable fluxes, to the action of a flame obtained by the combustion of pulverized coal in the necessary quantity of

superheated air, in order that the combustion produces carbon monoxide and a small quantity of carbonic acid in a proportion smaller than that of carbon monoxide.

The foregoing specification of my "Process for the direct reduction of ores, and particularly of iron ores", signed by me this 2nd day of February, 1923.

LUCIEN PAUL BASSET.